

## UNITED STATES PATENT OFFICE

2,365,386

## MAGNESIUM PRODUCTION

Robert A. Boyer, Dearborn, and Elbert E. Ensign, Ypsilanti, Mich., assignors to Ford Motor Company, Dearborn, Mich., a corporation of Delaware

No Drawing. Application September 12, 1942,  
Serial No. 458,128

12 Claims. (Cl. 75—67)

This invention relates to the production of magnesium by the thermal reduction of magnesium ores, and more particularly the production of magnesium by the ferrosilicon process aided by catalytic action.

Heretofore, metallic magnesium has been chiefly produced commercially by the electrolytic process involving a fused magnesium chloride bath. Although other processes such as the ferrosilicon reduction, carbon reduction and reduction by other metals have been greatly publicized, and although these processes have produced magnesium metal in laboratory experiments, they have been found to be economically unfeasible for large-scale production. In many cases the use of these processes has been restrained from commercial success by reason of unforeseen adverse conditions and difficulties that are inherent with large-scale production and lack of suitable equipment with the ability to withstand the stresses and strains imposed on it by the process. The ferrosilicon process has been one of those processes which has been so hampered. Satisfactory yield in this process is governed by temperature of the reaction since other conditions such as time and pressure can be more easily overcome. Thus, the temperature range at which the greatest efficiency is obtained is beyond the temperature range of the alloys which are used in constructing the equipment for the process.

The effect of the temperature gradient is clearly shown in the following chart in which the pressures and time elements are maintained relatively constant:

Temperature yield chart

|           | Percent yield |
|-----------|---------------|
| 2,000° F. | 4             |
| 2,100° F. | 9             |
| 2,200° F. | 40            |
| 2,300° F. | 45            |
| 2,400° F. | 65            |

From the above results, it is seen that theoretical yields are only approached at the higher temperatures. However, the heat and oxidation-resistant alloys such as nichrome are not suitable for the upper limits of the above temperature range since at the higher temperatures the effective life of the retort may be only several hours. Moreover, even though at lower temperatures the life is greatly increased the process also becomes economically unfeasible due to the extremely low yield obtainable.

It is therefore an object of this invention to produce improved efficiency in a ferrosilicon reduction of magnesium ores, said improvement to be effective throughout the temperature range 5 inherent of the process. Essentially, yields may be derived at a given temperature by this invention which, formerly, could only be obtained at a much higher temperature.

The data comprising temperature-yield chart 10 above was obtained from numerous tests which we choose to term as the "standard run." The standard run consists of a briquetted charge containing 81.6% of calcined dolomite and 18.4% of ferrosilicon which is maintained for 30 minutes at the reaction temperatures and at a pressure of from 50 to 150 microns. We propose to increase the efficiency of the above standard run by creating within the reaction 20 certain conditions which will bring about increased yield. This increased productivity occurs while the other factors such as temperature, time and pressure remain relatively constant; moreover, the yield may be increased at any given temperature range.

25 We have found that we may retard or accelerate the reaction of the ferrosilicon process such as to increase or decrease the yield. This is brought about by incorporating into the furnace charge certain catalytic agents producing 30 the desired effects. Catalytic agents which we have found to work successfully are:

|    | Negative catalytic agents                                                                             | Positive catalytic agents                                                                                    |
|----|-------------------------------------------------------------------------------------------------------|--------------------------------------------------------------------------------------------------------------|
| 35 | Oxides of iron<br>Sodium chloride<br>Calcium carbonate<br>Magnesium carbonate<br>Silica<br>Boric acid | Aluminum oxide<br>Beryllium oxide<br>Ceric oxide<br>Titanium dioxide<br>Zirconium oxide<br>Kyanite<br>Kaolin |
| 40 |                                                                                                       |                                                                                                              |
| 45 |                                                                                                       |                                                                                                              |

As it is the purpose of this invention to increase the efficiency of the ferrosilicon process, the negative catalytic agents may be disregarded. However, from this data one is able to predict the efficiency of the process when the charge contains such compounds even in very minute quantities.

Improvements in the production of magnesium processing, as pointed out by this invention, are best practiced in the conventional ferrosilicon process which consists chiefly of a tubular retort furnace whose ends may be sealed and may be maintained under reduced pressures. The tubular retort must be constructed of an alloy 50 having supreme heat-resisting and antioxida-

tion properties since it has been shown that the greatest yield may be obtained at the higher temperatures. The heating may be accomplished by conventional means such as external gas heating, glow bars, molten, fused baths and by other conventional means.

The charge of raw materials of this invention consists of the following:

|                   | Parts    |
|-------------------|----------|
| Calcined dolomite | 75 to 85 |
| Ferrosilicon      | 15 to 25 |
| Catalyst          | 1/2 to 5 |

The dolomite, ferrosilicon and catalyst in finely ground form are thoroughly mixed in the above ratios and then briquetted. The briquettes are then charged into a tubular retort and are subjected to temperatures of from 2,100 to 2,400° F. under a pressure of about 75 to 200 microns. A preferred form of the above formula comprises:

|                   | Parts |
|-------------------|-------|
| Calcined dolomite | 81    |
| Ferrosilicon      | 19    |
| Catalyst          | 1     |

The catalyst mentioned here is taken from the group consisting of aluminum oxide, beryllium oxide, ceric oxide, titanium dioxide, zirconium oxide, kyanite and kaolin. In many cases it has been found that 1/2 to 1% of a catalyst may be sufficient to cause said increase and that the additional catalyst would not produce greater increase in efficiency.

At this time the exact phenomenon that occurs within the reaction chamber due to the added foreign substances is not clearly understood. This reaction is of such a nature that no one, to our knowledge, has as yet seen fit to present an explanation. This type of complicated reaction in which a solid produces a catalytic reaction on another solid may probably be best interpreted in the light of interfaces as explained in "Treatise on Physical Chemistry," by Taylor. Taylor explains that the solid-to-solid interfacial activity or the catalytic action of one solid on another whereby a product of a different phase may be formed is not uncommon. As a further explanation of this in relation to our process it is thought these interfaces bring about a true equilibrium condition much faster. Thus in our case catalytic action occurs between a solid dolomite or other magnesium-bearing ores and a solid oxide or like catalyst to produce magnesium vapor while the residue remains in a solid state throughout the reaction.

Another explanation may be that there occurs among the ingredients a fusion and the fused product tends to hasten the liberation of magnesium by interfaces. This may be further explained by observing the reaction of some negative catalytic agent such as oxides of iron and silica and eliminating these negative catalysts by means of positive catalytic agents. It is generally believed that the two antagonistic catalysts fuse forming a complex compound which is neutral to the reaction or possibly retains its catalytic effects. However, since kyanite and kaolin exert positive catalytic action on the process and since these substances are complex compounds of a retardant  $SiO_2$  and an accelerator  $Al_2O_3$  it is believable that the accelerating effects predominate whenever a complex compound is formed by fusion of two antagonistic catalysts. The raw materials of the ferrosilicon process may contain retardants as impurities such as silica and iron oxide, the elimination of which is almost an

impossibility prior to processing. Therefore, it follows that the yield is increased by elimination of these retardants, or by the use of counteracting elements.

It should also be noted that the interfaces and other reactions of the process occur in the solid phase. The ability of the residue to remain in a solid state is of prime importance, particularly in the process using a horizontal tubular retort.

10 It would be extremely difficult to maintain a retort free from an insulating layer of residue if the charge were to become molten, or to charge and discharge the retort if the residue were likely to become tacky or gummy.

15 However, it has been suggested in U. S. Patent No. 2,224,160 that adding certain ingredients, which will reduce the melting temperature of the residue, is a decided advantage. This invention relates primarily to the maintenance of the slag through certain percentages having a low melting point, so that the residue may be removed in the molten state.

20 Our invention may be briefly summarized and differs from the above patent in that we incorporate in our charge a very small percentage of a catalytic agent whereby solid-to-solid interfaces between the magnesium-bearing ore and the reducing agent ferrosilicon occurs, thus increasing the yield and efficiency. We have attempted briefly to explain the physical or chemical phenomena in the solid-to-solid reaction when metallic oxides are used as catalysts or accelerators.

25 Other advantages will readily occur to those familiar with this art and it is the applicants' intention, although some changes may be made in the process described without departing from the spirit of our invention, to cover by our claims such claims as may easily be included within the scope of this invention.

30 We claim as our invention:

35 1. In the process for the production of metallic magnesium, a charge comprising magnesium bearing ore, ferrosilicon and a catalyst, said catalyst being one of aluminum oxide, beryllium oxide, ceric oxide, titanium dioxide and zirconium oxide, said charge subjected to a temperature of greater than 2,100° F. at a pressure of less than 1,000 microns.

40 2. In the process for the production of metallic magnesium a charge comprising:

|                   | Parts |
|-------------------|-------|
| Calcined dolomite | 75-85 |
| Ferrosilicon      | 15-25 |
| Catalyst          | 1/4-4 |

45 said catalyst being one of aluminum oxide, beryllium oxide, ceric oxide, titanium dioxide and zirconium oxide, said charge subjected to a temperature of greater than 2,100° F. at a pressure of less than 1,000 microns.

50 3. In the process for the production of metallic magnesium a charge comprising:

|                   | Parts |
|-------------------|-------|
| Calcined dolomite | 81    |
| Ferrosilicon      | 19    |
| Catalyst          | 1     |

55 said catalyst being one of aluminum oxide, beryllium oxide, ceric oxide, titanium dioxide and zirconium oxide, said charge subjected to a temperature of greater than 2,100° F. at a pressure of less than 1,000 microns.

60 4. In the process for the production of metallic magnesium a charge comprising calcined dolomite, ferrosilicon and  $Al_2O_3$ , said charge sub-

jected to a temperature of greater than 2,100° F. at a pressure of less than 1,000 microns.

5. In the process for the production of metallic magnesium a charge comprising calcined dolomite, ferrosilicon and  $TiO_2$ , said charge subjected to a temperature of greater than 2,100° F. at a pressure of less than 1,000 microns.

6. In the process for the production of metallic magnesium a charge comprising calcined dolomite, ferrosilicon and  $Al_2O_3 \cdot SiO_2$ , said charge subjected to a temperature of greater than 2,100° F. at a pressure of less than 1,000 microns.

7. The process for the production of metallic magnesium comprising a charge of magnesium-bearing ore, ferrosilicon and a catalyst, said catalyst being one of aluminum oxide, beryllium oxide, ceric oxide, titanium dioxide, and zirconium oxide, heating said charge in a sealed retort above 2,100° F. at a pressure of less than 1,000 microns to liberate magnesium vapors, withdrawing said vapors from said retort, and condensing said vapors to reguline magnesium.

8. The process for the production of metallic magnesium comprising a charge of:

|                   |         |
|-------------------|---------|
| Parts             |         |
| Calcined dolomite | 75-85   |
| Ferrosilicon      | 15-25   |
| Catalyst          | 1/4 - 4 |

said catalyst being one of aluminum oxide, beryllium oxide, ceric oxide, titanium dioxide and zirconium oxide, heating said charge in a sealed retort above 2,100° F. at a pressure of less than 1,000 microns to liberate magnesium vapors, withdrawing said vapors from said retort, and condensing said vapors to reguline magnesium.

9. The process for the production of metallic magnesium comprising a charge of:

|                   |    |
|-------------------|----|
| Parts             |    |
| Calcined dolomite | 81 |
| Ferrosilicon      | 19 |
| Catalyst          | 1  |

15 said catalyst being one of aluminum oxide, beryllium oxide, ceric oxide, titanium dioxide and zirconium oxide, heating said charge in a sealed retort above 2,100° F. at a pressure of less than 1,000 microns to liberate magnesium vapors, withdrawing said vapors from said retort, and condensing said vapors to reguline magnesium.

10. The process of claim 8 in which the catalyst is  $Al_2O_3$ .

11. The process of claim 8 in which the catalyst is  $TiO_2$ .

12. The process of claim 8 in which the catalyst is  $Al_2O_3 \cdot SiO_2$ .

ROBERT A. BOYER,  
ELBERT E. ENSIGN.